

# United States Patent Office

2,742,341

Patented Apr. 17, 1956

1

2,742,341

## AFTERTREATMENT OF AZOIC-DYED CELLULOSE DERIVATIVES

Earl L. Youse, Port Huron, Mich., and Donald E. Mar-  
non, Glen Rock, N. J., assignors to General Aniline &  
Film Corporation, New York, N. Y., a corporation of  
Delaware

No Drawing. Application April 30, 1952,  
Serial No. 285,314

2 Claims. (Cl. 8—48)

This invention relates to improvements in the dyeing of materials containing an organic derivative of cellulose with azo dyes whereby improved colorations of good fastness are obtained without objectionably tendering the dyed materials; and more particularly, it relates to a treatment of azo dyed cellulose acetate textile materials of off-shade color and poor lightfastness by subjecting these materials to a treatment at a temperature in the range of 120° to 190° F. for a time in the range of 3 to 30 minutes with an aqueous solution containing about 0.5 to 10% of a polar organic swelling agent for the cellulose derivative, using 10 to 40 parts by weight of the solution per part of the textile material, and selecting the temperature, time, concentration and amount of solution used so as to develop the true color of the dye as compared to the color obtained therewith on cotton, and simultaneously improve its lightfastness.

The azo dyes are particularly desirable for dyeing cellulose acetate and the like textile materials inasmuch as they provide desirable bright colors which are impervious to so-called gas-fading. However, the colors obtained thereon by the usual ingrain dyeing methods are of off-shade color as compared to the colors obtained with the same dyes on cotton; and in many cases they have very poor lightfastness.

Attempts have been made heretofore to provide azo dyed cellulose acetate materials by treating the dyed material with a very high concentration of a swelling agent for the cellulose acetate or by treatment at a very high temperature, such as 100° C. It has been found that such treatments are reflected in a very objectionable tendering of the textile material.

It has been found in accordance with the invention that the above discussed drawbacks may be overcome and azo dyed materials containing an organic derivative of cellulose may be provided having true color and good fastness properties without objectionably tendering the materials.

The objects achieved in accordance with the invention include the provision of a process of treating azo dyed materials containing an organic derivative of cellulose and having an off-shade color and poor lightfastness by subjecting these materials to a treatment at a temperature in the range of 120° to 190° F. for a time in the range of 3 to 30 minutes with an aqueous solution containing about 0.5 to 10% of a polar organic swelling agent for the cellulose derivative, using 10 to 40 parts by weight of the aqueous solution per part of the dyed material, and selecting the time, temperature, concentration and amount of solution so as to develop the true color of the dye and improve its lightfastness without objectionably creasing the material; the provision of such a process applied to textile material containing cellulose acetate; the provision of such a process wherein the swelling agent is a mixture of about 3 to 7% by weight of phthalic anhydride in a water-sol-

2

uble phenol; the provision of such a process wherein the swelling agent is ethylene glycol monobutyl ether; the provision of such a process wherein the swelling agent is furfural; the provision of such a process wherein the swelling agent is pyridine; the provision of such a process wherein the swelling agent is epichlorohydrin; and other objects which will be apparent as details or embodiments of the invention are set forth hereinafter.

In order to facilitate a clear understanding of the invention, the following preferred specific embodiments are described in detail.

For one part by weight of cellulose acetate fabric the following baths are prepared:

- 15 20 parts water  
3% guanidine carbonate (on the weight of the fabric)  
3% sodium naphthalene-sulfonate;  
then thereto add:  
20 3% of 2,3-hydroxy-naphthoic acid anilide (previously brought into solution in about 10% sodium hydroxide in ethanol).

Then a dispersion of 6% of 4-benzoylaminio-2,5-dimethoxy aniline in water is prepared (using molecular proportions of the amine and water) and added to the above bath, which is then heated to 120° F.

The cellulose acetate fabric is then introduced into this bath and treated therein for 45 minutes at 160° F., after which it is washed with cold water. Then the fabric

30 is treated with:  
2% sodium nitrite (on the weight of the fabric) in 10% of 56% aqueous acidic acid

for 30 minutes at 75° F. and then 30 minutes at 160° F. Following this it is washed and then dried.

The dyed cloth was of an undesirable violet off-shade color, and its lightfastness on exposure to light (in a Fade-Ometer) was only 10 hours.

A similarly dyed cellulose acetate fabric was subjected to a treatment at 180° F. for 7 minutes in the following bath (per part by weight of the dyed fabric):

- 20 parts distilled water  
.25 part of a 5.5% mixture of phthalic anhydride in phenol  
45 0.1 part of polyoxyethylated nonyl phenol containing about 8 oxyethyl groups;

and washed and dried.

The resulting material was of a desirable true blue color (compared with the color obtained with this dye on cotton), and it showed a lightfastness of 40 hours in the above-described test. A very desirable feature of the blue dyed material is its imperviousness to fading in the presence of acidic gases, inasmuch as this is 55 a well-known disadvantage of many of the commercial dyestuffs for cellulose acetate.

The desirable blue colored fabric obtained by this process has substantially the same strength properties as the undyed fabric. This is noteworthy when one considers that subjecting the off-colored cloth to a treatment at the boil can give the desired blue shade, but this treatment results in a very objectionable creasing of the textile fibers. The inclusion of phthalic anhydride with the phenol avoids the objectionable tendering of the fibers which is known to occur when phenol alone is used, especially at higher concentrations.

Comparable results to the foregoing are achieved using various modifications, such as the following. Other azo dyes which present a similar problem when ingrain dyed as described hereinabove are those prepared from 4-benzoylaminio-2,5-dimethoxy-aniline, 2-chlor-4-benzoylaminio-5-methoxy-aniline, 6-benzoylaminio-4-methoxy-3-

aminotoluene, 4-amino-4'-methoxy-diphenylamine, and amino-azotoluene, and similar amines or bases when coupled with a 2,3-hydroxy-naphthoic acid anilide, or o-toluidide, or o-anisidine, or 2,3-hydroxyanthracene-carboxylic acid, and the like. Generally, the dyes which give true colors or blue shades initially have an off-color of a reddish or purplish hue; the dyes which have a green true color initially have a yellow or brown tinted off-shade; and the dyes which give a brown true color initially have a reddish off-shade. The invention is applicable to materials containing an organic derivative of cellulose such as cellulose acetate, formate, propionate, butyrate, or mixed acetate propionate or mixed acetate butyrate, methyl ethyl or benzyl cellulose, and the like. The material may be in the form of films, fibers, yarns, fabrics or filaments. In the case of textile materials, the material may be made entirely of the cellulose derivative or it may be a mixed material which also contains cotton, natural silk, viscose rayon, or wool.

The temperature and other conditions for treating the dyed material should be such as to achieve the desired color improvement effect and at the same time avoid objectionable creasing of the material being treated. A desirable temperature range is 120° to 190° F., preferably 140° to 180° F. The treatment time may be in the range of 3 to 30 minutes. The aqueous solution should contain from about 0.5 to 10% by weight of a polar organic swelling agent for the organic derivatives of cellulose, based on the weight of the latter; and the bath should contain an amount in the range of 10 to 40 parts by weight of the aqueous solution per part of the dyed material. With the higher concentrations and relatively larger amounts of the solution, the color improvement effect may be obtained at lower temperature or treatment time. With the lower concentrations and proportions of the solution used the higher treating temperatures or longer treating times within the above ranges may be required to achieve the desired color improvement. In any combination within the above ranges, the treating conditions should not be sufficiently strenuous to objectionably crease the cellulose derivative material.

Although the effect achieved with the above-mentioned mixture of phthalic anhydride with phenol is regarded as particularly unique, desirable results may be obtained with many other chemically inert swelling agents for the cellulose derivative; and for cellulose acetate fabrics, such swelling agents as ethylene glycol monobutyl ether, furfural, pyridine and epichlorohydrin give desirable results

when used under the above conditions. Instead of phenol in the above-described mixed swelling agent, other water-soluble phenolic materials may be used, such as cresol, xylol and the like. Other equivalent surface-active agents may be substituted for the polyoxyethylated nonyl phenol used in the above-described bath, such as are conventionally used in dyeing treatments.

In view of the foregoing disclosures, variations and modifications of the invention will be apparent to one skilled in the art, and it is intended to include within the invention all such variations and modifications except as do not come within the scope of the appended claims.

We claim:

1. In the process of ingrain dyeing of textile materials containing an organic derivative of cellulose with an azo dye whereby an off-shade color is obtained, compared to the true color obtained with said dye on cotton, the improvement which comprises subjecting the thus dyed material to a treatment at a temperature in the range of 120° to 190° F. for a time in the range of 3 to 30 minutes with an aqueous solution containing about 0.5 to 10% of a polar organic swelling agent for the cellulose derivative, said organic swelling agent comprising a mixture of about 3 to 7 per cent by weight of phthalic anhydride in phenol, using 10 to 40 parts by weight of the aqueous solution per part of the dyed material, the temperature, time, concentration and amount of solution being selected so as to develop the true color of the dye and improve its light-fastness without objectionably tendering the textile material.

2. The process of claim 1 operated at about 180° F. for 7 minutes using about 20 parts of an aqueous solution containing about 0.5% of polyoxyethylated nonyl phenol containing about 8 oxyethyl groups and 1.14% of phthalic anhydride in phenol per part of cellulose acetate fabric dyed with diazotized 4-benzoylamino-2,5-diethoxy aniline coupled with the anilide of 2,3-hydroxy-naphthoic acid.

#### References Cited in the file of this patent

#### UNITED STATES PATENTS

|           |             |               |
|-----------|-------------|---------------|
| 961,241   | Knoevenagel | June 14, 1910 |
| 2,048,786 | Ellis       | July 28, 1936 |
| 2,643,175 | Salvin      | June 23, 1953 |

#### OTHER REFERENCES

British Rayon and Silk Journal for October 1950, page 48.